

# United States Patent Office

2,860,972

Patented Nov. 18, 1958

1

2,860,972

## MOLYBDENUM-COBALT-NICKEL ALLOY

William M. Fraser, Cedar Grove, N. J., assignor to Westinghouse Electric Corporation, East Pittsburgh, Pa., a corporation of Pennsylvania

No Drawing. Application July 2, 1956  
Serial No. 595,045

2 Claims. (Cl. 75—176)

This invention relates to alloys and, more particularly, to an alloy of molybdenum, cobalt and nickel.

Heretofore, high-strength alloys for tool steels and similar applications have comprised tungsten carbides and high-speed tool steels, among others. While the tungsten carbides are very suitable from the standpoint of hardness, they are difficult to fabricate and sharpen, necessitating grinding with diamond bits because of their extreme hardness. High-speed tool steels are considerably softer than tungsten carbides and may be easily ground with conventional aluminum oxide or silicon carbide grinding wheels, but their relatively low hardness and other physical properties do not enable these materials to stand up very well when cutting very hard materials.

It is the general object of this invention to avoid and overcome the foregoing and other difficulties of and objections to prior art practices by the provision of a molybdenum-cobalt-nickel alloy which combines some of the desirable properties of high-speed tool steel with some of the desirable properties of tungsten carbide.

The aforesaid object of the invention, and other objects which will become apparent as the description proceeds, are achieved by providing permissible constituent ranges and optimum composition for an alloy of molybdenum, cobalt and nickel.

Although the uses of the alloy herein described are broadly applicable to any type of tool or equipment where hardness, high wear resistance and strength are important, such as drawing and extrusion dies, mandrels, gauges, guide rings, drills, forming tools, circular saws, reamers, counter bores, etc., the alloy is particularly adapted for use as a tool bit and hence its properties as applied to this use will be described.

Basically the alloy consists of a ternary alloy of molybdenum, cobalt and nickel wherein the cobalt is present in amounts from 2.5% to 6% by weight of the alloy and the nickel is present in amounts from 0.1% to 0.7% by weight of the alloy, with the balance being molybdenum. Thus the molybdenum may be present in amounts of from 93.3% to 97.4% by weight of the alloy. The preferred composition for the alloy is about 96.5% by weight molybdenum, about 3% by weight cobalt and about 0.5% by weight nickel.

A binary alloy of molybdenum and cobalt within the ranges as specified will be quite hard and wear resistant, but will display a tendency for sudden failure under stress. That is, when the alloy fails under stress it will develop very large fractures with the possibility of flying fragments, which is of course undesirable. It has been found that the addition of nickel, within the ranges as specified, eliminates this tendency toward sudden failure and the ternary alloy will wear or at most tend to chip off in small flakes rather than display the sudden-fracture type of failure. If less than 0.1% by weight of nickel is used, this sudden-failure defects of the molybdenum-cobalt binary alloy is not substantially eliminated.

2

and if more than 0.7% by weight of nickel is utilized in the ternary alloy, the alloy hardness is decreased.

Regarding the cobalt component of the ternary alloy, if less than 2.5% by weight of cobalt is utilized, the alloy is not sufficiently hard and if more than 6% by weight of cobalt is utilized, the alloy has some tendency to become brittle, thereby limiting its usefulness as a tool bit, for example.

In fabricating the molybdenum-cobalt-nickel alloy, 10 molybdenum dioxide may be admixed with cobalt and nickel acetate in such proportions that the metallic content of the components of the mixture corresponding to the desired percentages of each compound in the final alloy. These materials are preferably thoroughly admixed by means of a water slurry, after which the water is dried off leaving a very even mixture of molybdenum dioxide and the finely-divided cobalt and nickel acetates. This dried material is then reduced to finely-divided metallic form by reduction in a hydrogen atmosphere at 15 a temperature of 1100° C. for about 6 hours. The reduction temperature may vary from 1000° C. to 1200° C., for example, the lower the temperature the longer the period of reduction.

The reduced metal thus comprises a very even admixture of the elements of the ternary alloy in amounts corresponding to the final composition of the alloy. The finely-divided powders comprising this admixture are then compressed into a green ingot of the desired configuration. This green ingot is sintered under non-20 oxidizing conditions at a temperature of from 1550° C. to 1660° C. for from 1 to 3 hours. As a specific example, the sintering temperature may be 1600° C. for a period of 2 hours in a hydrogen atmosphere. The preferred atmosphere for sintering is a hydrogen atmosphere 25 although any other non-oxidizing conditions would be suitable.

After sintering, the ingot is age-hardened by maintaining it under non-oxidizing conditions at a temperature of from 650° C. to 750° C. for a period of from 40 4 to 24 hours, although the preferred temperature for age-hardening is about 700° C. for a period of from 8 to 12 hours. The preferred atmosphere for age hardening is hydrogen.

If molybdenum dioxide is not available, the trioxide 45 may be reduced to dioxide by prefiring at a temperature of about 550° C. to 650° C. for a period of about 6 hours, for example. If the molybdenum trioxide is utilized and is first reduced to the dioxide, it is preferable to add the other constituents of the alloy after the first preliminary reduction to the dioxide, although the alloy constituents may be added directly to the trioxide if desired, before the first reduction to the dioxide. Also, it is desirable, although not mandatory, to screen the finely-divided metallic material through a 40 mesh screen 50 (see A. S. T. M. Designation: E11-39) after reduction to the metallic state and before formation of the green ingot.

In the foregoing method, cobalt and nickel acetate 55 have been given as specific examples. These materials are not meant to be limiting and any water-soluble salts of cobalt and nickel which can be readily decomposed to a residue of cobalt and nickel powders respectively under high-temperature reducing conditions may be utilized, and cobalt nitrate and nickel nitrate would be as acceptable as the acetates, if it is desired to use these compounds in forming the slurry.

It is possible to mix finely-divided molybdenum, cobalt 60 and nickel directly in the prescribed proportions, prior to forming the green ingot, thus eliminating any reducing steps. However, the finely-divided metallic powders normally cannot be mixed as thoroughly as with

the water-slurry method. Thus the preferred method of forming the metallic powder admixture, prior to forming the green ingot, is the aforementioned water slurry technique.

After the alloy has been age-hardened, it is very hard and cannot be machined as a practical matter, but must be ground to the desired configuration. Since grinding is a fairly slow and expensive process as compared to machining, it may be desirable to prefire the green ingot at a temperature of from 800° C. to 1000° C. for a period of 1 to 2 hours, for example. In this stage, the green ingot has sufficient strength to enable it to be machined readily, but is not sufficiently hard as to make machining difficult. After this prefire, the machine ingot may be sintered and age hardened under conditions as hereinbefore specified.

The physical and mechanical properties of the molybdenum-cobalt-nickel alloy specified are excellent with respect to the requirements of high-speed tool bits. For purposes of comparison, the physical and mechanical properties of this alloy can be compared to a tungsten carbide tool bit having a composition of 94% tungsten carbide and 6% cobalt and a high speed tool steel having as composition 18% tungsten, 4% chromium, 1% vanadium, 0.7% carbon and the remainder iron. These property comparisons will be examined in the following paragraphs.

With respect to hardness, the molybdenum-cobalt-nickel alloys display a Rockwell hardness of 60-62 which is comparable to the Rockwell hardness of high-speed tool steel. This is somewhat less than the hardness of tungsten carbide which displays a Rockwell hardness of from 76 to 80. This relatively low hardness as compared to tungsten carbide has both advantages and disadvantages. For example, the relatively low hardness means that the tools can be easily ground with conventional grinding wheels whereas the tungsten carbide must be ground with diamond wheels, although the relatively low hardness with respect to tungsten carbide would seem to indicate that the ternary alloy would not stand up as well when cutting very hard materials. However, another factor enters into this, for the hardness at high temperatures, which is most important in high-speed cutting tools, is apparently very good for the ternary alloy as compared to tungsten carbide which softens rapidly above 900° C. and high speed tool steels which soften rapidly above 700° C. The results of the actual machining tests conducted would seem to indicate that the molybdenum-cobalt-nickel alloy has excellent high-temperature characteristics.

The modulus of elasticity for the ternary alloy was found to be about  $41.5 \times 10^6$  p. s. i. while the modulus for the high speed tool steel was  $31.5 \times 10^6$  and the modulus for tungsten carbide was measured as  $88 \times 10^6$ . It should be noted that a high modulus is desirable in a cutting tool to minimize the elastic deflection of the tool and thereby obtain machining accuracy.

The thermal expansion and thermal conductivity for the ternary alloy were found to be about  $5.08 \times 10^{-6}$  (per °C.) and 0.12 (cal. cm.<sup>-1</sup> sec.<sup>-1</sup> 0 C.<sup>-1</sup>) respectively, compared to  $5 \times 10^{-6}$  and 0.19 for tungsten carbide. This

is to be compared with a thermal coefficient of  $11.23 \times 10^{-6}$  and a thermal conductivity of 0.058 for the high speed tool steel. It should be noted that a low thermal expansion and a high thermal conductivity are very desirable in a tool material, since the former permits more accurate machining and since the latter permits heat conduction from the tool tip and thereby helps keep down tool-tip temperatures.

In actual cutting tests, the high-speed tool steel and carbide-tipped tool were mounted in a turret along with the ternary alloy in order to machine a 2" diameter bar of austenitic stainless steel, with the dimensions of all of the tips being the same. Under a fairly light load all of the bits held up equally well and there was so marked evidence of wear or other type of failure. In order to test the individual tools to failure, a second series of machining tests was made in which the feed and depth of the cut was held constant and the cutting speed increased until failure of the bit occurred or until the lathe stalled. In this test, the high-speed tool steel bit failed at relatively low cutting speeds. The tungsten carbide tipped bit and the molybdenum-cobalt-nickel alloy bit withstood the highest cutting speeds obtainable with the lathe used for the test and the lathe stalled before the bits failed. However, the tungsten carbide bit showed evidence of rapid wear at the highest cutting speed and the molybdenum-cobalt-nickel alloy bit did not show any evidence of wear, indicating excellent high temperature hardness. While this foregoing test is of a qualitative nature, it indicates the excellent characteristics of the molybdenum-cobalt-nickel alloy as a cutting tool and this is borne out by the measured physical and mechanical properties of this alloy.

It will be recognized that the objects of the invention have been achieved by providing a molybdenum-cobalt-nickel alloy having high hardness, high wear resistance and strength.

While this alloy appears particularly desirable for use in high speed tool bit applications it should be mentioned again that it should also be useful in many other types of applications where its hardness, strength and wear resistance make its use desirable.

While in accordance with the patent statutes, one best-known embodiment of the invention has been illustrated and described in detail, it is to be particularly understood that the invention is not limited thereto or thereby.

I claim:

1. A metallic alloy containing from 93.3% to 97.4% by weight of molybdenum, from 2.5% to 6% by weight of cobalt, and from 0.1% to 0.7% by weight of nickel.
2. A metallic alloy containing about 96.5% by weight of molybdenum, about 3% by weight of cobalt, and about 0.5% by weight of nickel.

55 References Cited in the file of this patent

UNITED STATES PATENTS

2,467,675 Kurtz et al. ----- Apr. 19, 1949

60 FOREIGN PATENTS  
462,214 Canada ----- Jan. 3, 1950